

S. McLOUD.

SPRING.

APPLICATION FILED FEB. 19, 1917.

1,250,332.

Patented Dec. 18, 1917.



Witness:

R. S. Dillingham

Invention:  
By Sidney McCloud,  
Att'y  
J. Fortune King -

# UNITED STATES PATENT OFFICE.

SIDNEY McCLOUD, OF SOUTH CHICAGO, ILLINOIS.

## SPRING.

1,250,332.

Specification of Letters Patent. Patented Dec. 18, 1917.

Application filed February 19, 1917. Serial No. 149,430.

To all whom it may concern:

Be it known that I, SIDNEY McCLOUD, a citizen of the United States, residing at South Chicago, Cook county, State of Illinois, have invented certain new and useful Improvements in Springs, of which the following, taken in connection with the drawing, is a description.

My invention has for its object the production of a resilient bar or spring of metal formed of a plurality of thicknesses which have been bent, folded and overlapped and compressed together by passing them through rollers or the like while the metal is in a more or less heated state at less than a welding heat.

A further object of my invention is to produce an article of this kind by means of which I am able to overcome certain imperfections found in metals as now made, even of the best steel or iron, which contain portions having a lack or an excess of carbon, thereby rendering the material brittle in such portions and easily liable to break, and when cracked or broken the entire article has to be discarded as useless.

A further object of my invention is to produce a single bar of metal so bent, folded and overlapped as to present a plurality of thicknesses superposed one above the other out of which such articles as leaf springs, for instance, may be formed. By my construction each spring will have a plurality of layers which will extend from end to end of the article and be shaped to give strength where strength is needed, at the same time to afford the resiliency desired in the use of such an article and always present greater tensile and compression strength than is possible with a bar of metal formed of a solid piece.

In the accompanying drawing, I have illustrated what I now consider the best form of my construction, although it is obvious it may be employed in other constructions than this form of spring, and in this drawing,

Figure 1 is a side elevation of my construction utilized in a leaf spring;

Fig. 2 is a longitudinal, sectional view of a portion of the spring; and

Fig. 3 is a transverse, sectional view of the same.

In forming bars of this character I first provide a sheet of metal which is rolled the desired length and thickness and at the

point of bending is rolled slightly thinner in cross section than elsewhere. This facilitates the bending operation and permits the parts to be closely compressed together in the shape desired.

Referring to the drawing, A represents the side of a leaf spring which is formed in the manner described and in which the sheet of metal has been rolled thinner at the outer ends thereof than at the center where the greater strength is required. The folds of this material may be bent in various ways. In Fig. 3 I have shown a single sheet bent and overlapped to form five thicknesses in cross section, with both ends a of the metal folded inside the bar.

The plate forming the spring is rolled while hot and the rolls arranged so that the plate will have longitudinal lines for bending the material which are thinner in cross section, as at a', than are the laminations forming the bar.

After the material has been bent and folded along longitudinal lines it is further compressed in the rolls until the different laminations are pressed closely together, as shown in Figs. 2 and 3, the several laminations being in contact with each other but not welded together at any point.

The bar may be further compressed in the rolls to elongate the material in the form desired for an article of manufacture, such as a leaf spring, with the outer ends thereof B reduced in thickness, as shown in the drawing. In this case, each of the laminations extend to the ends of the bar and present the desired resiliency and flexibility of each plate or lamination of the material.

I do not wish to be limited to the manner of folding the material as here shown, as it is obvious it may be bent and compressed together in the form of corrugations or in any other manner which would present a flat surface or bar having a plurality of laminations in its thickness, the idea being to provide a flat bar of material formed of a plurality of thicknesses extending from end to end thereof, so bent, folded and overlapped as to have the outward appearance of a single bar, but which is in reality made up of a number of folds or sections bent and overlapped together as shown.

In the formation of bars of this kind I wish to be understood as contemplating the folding of two or more plates laid upon each other before bending and overlapping

in the manner shown, as well as the use of a single plate as here described.

I claim:

1. As a new article of manufacture, a spring formed of a sheet of material which is bent, folded and overlapped upon itself in contacting relationship to form a flat surface, substantially as described.
2. As a new article of manufacture, a spring formed of a sheet of metal, which is thinner in cross section along certain separated longitudinal areas than is the body of the sheet, the sheet being bent or folded along such areas to overlap the adjacent portions of the body of the sheet into contacting relationship to form a bar.
3. As a new article of manufacture, a spring formed of a sheet of metal bent, folded and overlapped to form a plurality of laminations compressed closely but not welded together, substantially as described.
4. As a new article of manufacture, a

spring formed of a sheet of metal bent, folded and overlapped to form a plurality of laminations compressed closely but not welded 25 together, each lamination extending from end to end of the material, substantially as described.

5. As a new article of manufacture, a spring formed of metal bent and folded into 30 a plurality of laminations with the edges thereof unexposed, substantially as described.

6. As a new article of manufacture, a spring formed of metal having a plurality 35 of laminations bent, folded and overlapped upon each other and compressed into contacting relationship to present a folded surface, but with said laminations not welded together, substantially as described. 40

In testimony whereof I have signed this specification.

SIDNEY McCLOUD.

Copies of this patent may be obtained for five cents each, by addressing the "Commissioner of Patents, Washington, D. C."